

Oct. 21, 1947.

F. A. MARTY

2,429,271

MASKING PAPER SUCH AS FOR LITHOGRAPHY

Filed Nov. 16, 1944



LAYER 1, RELATIVELY TRANSPARENT  
SHEET OF PAPER DYED AN ORANGE TO A  
YELLOW COLOR;

LAYER 2, MIXTURE OF SILICATE OF SODA  
WITH AN EQUALIZER MATERIAL SUCH AS  
GELATIN OR LATEX;

LAYER 3, CLAY IN SIZING SUCH AS CASEIN  
OR STARCH;

LAYER 4, MIXTURE OF SILICATE OF SODA  
WITH AN EQUALIZER SUCH AS GELATIN OR  
LATEX.

INVENTOR

Frank A. Marty

BY

Bohlbrue, Jasseff & Montstream

ATTORNEYS

## UNITED STATES PATENT OFFICE

2,429,271

MASKING PAPER SUCH AS FOR  
LITHOGRAPHY

Frank A. Marty, Flushing, N. Y.

Application November 16, 1944, Serial No. 563,807

6 Claims. (Cl. 88—109)

1

The invention relates to a paper designed particularly as a masking paper for lithographic stripping. In the layout of lithographic work, a negative is held in a desired position by a masking sheet and the desired extent of the negative to be printed on the lithographic plate is determined by cutting out or stripping the paper to the desired dimensions, shape and in its desired position. Such a lithographic masking sheet must be sufficiently transparent to the light from an incandescent lamp so that the matter or negative to be lithographed will be clearly visible therethrough for the layout and yet be impenetrable to the lithographic printing light such as a mercury vapor lamp.

It is an object of the invention to construct a lithographic masking paper particularly suitable for lithographic work.

Another object of the invention is to construct a masking sheet for lithographic work the color of which is sealed in and will not rub off.

Another object is to provide a masking sheet to which Scotch tape or other adhesive strip will adhere thereto and yet will readily pull off from the sheet.

Another object is to construct a masking sheet which will readily take pen ink, pencil or litho ink marks and lines.

A still further object is to construct a masking sheet which does not shrink or stretch under the usual conditions existing where lithographic work is done.

Other objects of the invention will appear more fully from the following description and the accompanying drawing in which the figure illustrates an enlarged portion of a masking sheet.

The masking paper of the invention utilizes a base sheet 1 which is orange or yellow in color because these colors are impenetrable to light used for lithographic work such as the mercury vapor lamp. The dye of the base sheet should be insensitive to alkali. This base sheet is preferably first coated with a mixture of silicate of soda with an equalizer material such as gelatin or latex in the proportions of about one part of water glass to nine parts of equalizer. This first coat 2 could be dispensed with although it improves the characteristics of the sheet so far as stretching and shrinking is concerned and also improves the cutting properties to give a sharp clear cut edge. The proportions of silicate of soda and an equalizer will vary with the type of paper used for example the proportion referred to is that best suited for ground wood paper and increasing amounts for the following in the order named, 55

2

sulphite, sulphate, sulka, rags, and combination of rags. The equalizer is used to give the sheet greater flexibility or to make the sheet less brittle.

5 A coating 3 of clay with a sizing such as casein or starch is next applied to the sheet. The clay is preferably a white clay which softens the yellow or orange to a pastel shade, and hence is less glaring upon the eyes. A hardening agent, such as formaldehyde, may be used in the clay mixture to harden the clay coating so that it does not chalk off of the sheet. The amount of formaldehyde used will vary and for best results enough is used so that the sheet will withstand a seven point or pick wax test of the surface. An equalizer may also be used with the clay coating to render the sheet less brittle.

10 A third coating 4 is applied to the sheet over the clay coating which is made up of a mixture of silicate of soda with an equalizer preferably in the proportions of about seven and one half parts of silicate of soda and two and a half parts of equalizer for best results. There may be considerable variation in these proportions.

15 The sheet which results is largely resistant to moisture and temperature and retains its dimensions with no or slight stretch or shrinkage irrespective of changes in humidity of the atmosphere or when subject to the heat from a lighted stripping table.

20 The sheet is transparent to ordinary light so that a negative which is secured to the under side of the sheet may be clearly seen therethrough. The pastel salmon color brings out the lines on the underlying negative

25 with clear cut lines through the masking sheet and is restful to the eyes. The surface of the sheet is of such character that Scotch tape and other adhesives will readily stick thereto to hold a negative in place upon the sheet, and yet the

30 surface permits easy removal of the Scotch tape and relatively free removal of other adhesive strips. The surface also is of such character that it can be written on with pencil, ordinary ink or litho ink.

35 40 45 The treatment seals in the dye of the base sheet with the result that smearing of the dye of the stock sheet cannot occur. Furthermore the kerosene used with paper negatives does not affect the transparency of the paper nor smear the dye of the base sheet which is sealed in by the coatings. Likewise oil or grease will not cause translucency of the paper.

This invention is presented to fill a need for improvement in a masking paper. It is understood that various modifications may and often

do occur to those skilled in the art, especially after benefiting from the teachings of an invention. Hence, it will be understood that this disclosure is illustrative of preferred means of embodying the invention in useful form by explaining the construction, and advantages thereof.

What is claimed is:

1. A lithographic masking paper comprising a stock sheet dyed an orange to a yellow color which is relatively transparent and the dye of which is insensitive to alkali, a coating of a mixture of clay and a sizing upon the sheet of stock, and a coating of a mixture of silicate of soda and an equalizer over the clay coating.

2. A lithographic masking paper comprising a stock sheet dyed an orange to a yellow color which is relatively transparent and the dye of which is insensitive to alkali, a coating upon the stock sheet including a mixture of silicate of soda and an equalizer, a coating of clay mixed with a sizing over the first coating, and a second coating of a mixture of silicate of soda and an equalizer over the clay coating.

3. A lithographic masking paper comprising a stock sheet dyed an orange to a yellow color which is relatively transparent and the dye of which is insensitive to alkali, a coating upon the paper of a mixture of silicate of soda and an equalizer, a coating of clay mixed with sizing and a hardening agent, and a second coating of a mixture of silicate of soda with an equalizer.

4. A lithographic masking paper comprising a stock sheet dyed an orange to a yellow color which is relatively transparent and the dye of which is insensitive to alkali, a coating upon the paper of a mixture of about one part of silicate of soda

and nine parts of an equalizer, a coating of clay mixed with sizing and a hardening agent, and a second coating of a mixture of about seven and a half parts of silicate of soda and two and a half parts of an equalizer.

5. A lithographic masking paper comprising a stock sheet dyed an orange to a yellow color which is relatively transparent and the dye of which is insensitive to alkali, a coating of white clay mixed with a sizing and a hardening agent upon the sheet, and a coating of a mixture of about seven and a half parts of silicate of soda and two and a half parts of an equalizer over the clay coating.

10 6. A lithographic masking paper comprising a stock sheet dyed an orange to a yellow color which is relatively transparent and the dye of which is insensitive to alkali, a coating upon the paper of a mixture of about one part of silicate of soda and nine parts of an equalizer, a coating of white clay mixed with sizing and a hardening agent, and a second coating of a mixture of about seven and a half parts of silicate of soda and two and a half parts of an equalizer.

15 25 FRANK A. MARTY.

#### REFERENCES CITED

The following references are of record in the file of this patent:

#### UNITED STATES PATENTS

| Number    | Name          | Date          |
|-----------|---------------|---------------|
| 2,043,860 | Morgan        | June 9, 1936  |
| 2,062,179 | Hunter        | Nov. 24, 1936 |
| 2,327,380 | Toland et al. | Aug. 24, 1943 |
| 2,361,665 | Toland et al. | Oct. 31, 1944 |